

A. E. GREENE.

PROCESS AND APPARATUS FOR EXTRACTING AND REFINING METALS AND ALLOYS.

APPLICATION FILED OCT. 25, 1909.

1,031,257.

Patented July 2, 1912.

4 SHEETS—SHEET 1.



Witnesses:

Geo. O. Davison  
Maurice Goldberger.

Inventor:

Albert E. Greene  
By Barton & Folk,  
Attest.

A. E. GREENE.

PROCESS AND APPARATUS FOR EXTRACTING AND REFINING METALS AND ALLOYS.

APPLICATION FILED OCT. 25, 1909.

1,031,257.

Patented July 2, 1912.

4 SHEETS—SHEET 2.



Witnesses:

R. D. Garrison  
Maurice Goldberger.

Inventor:

Albert E. Greene  
By Barton & Folk,  
Atty.

A. E. GREENE.

PROCESS AND APPARATUS FOR EXTRACTING AND REFINING METALS AND ALLOYS.  
APPLICATION FILED OCT. 25, 1909.

1,031,257.

Patented July 2, 1912.

4 SHEETS—SHEET 3.

Fig. 4



Fig. 5



Fig. 6



A. E. GREENE.

PROCESS AND APPARATUS FOR EXTRACTING AND REFINING METALS AND ALLOYS.

APPLICATION FILED OCT. 25, 1909.

1,031,257.

Patented July 2, 1912.

4 SHEETS-SHEET 4.



Witnesses

Geo. C. Davis  
Maurice Goldberger.

Inventor:  
Albert E. Greene  
By Barton & Folk  
Attest.

# UNITED STATES PATENT OFFICE.

ALBERT E. GREENE, OF CHICAGO, ILLINOIS.

## PROCESS AND APPARATUS FOR EXTRACTING AND REFINING METALS AND ALLOYS.

1,031,257.

Specification of Letters Patent.

Patented July 2, 1912.

Application filed October 25, 1909. Serial No. 524,298.

*To all whom it may concern:*

Be it known that I, ALBERT E. GREENE, citizen of the United States, residing at Chicago, in the county of Cook and State of Illinois, have invented a certain new and useful Improvement in Processes and Apparatus for Extracting and Refining Metals and Alloys, of which the following is a full, clear, concise, and exact description.

10 My invention relates to a process and apparatus for extracting and refining metals and alloys in general, and more particularly such metals as copper and iron.

15 It is especially applicable to the production of low-carbon steel.

The object of the invention is to provide a furnace of such construction as will permit of the usual treatment of the metal to whatever extent is desirable and will then 20 permit of such additional combined electrical and gaseous treatment as may be necessary to produce the required product.

As a process one feature of the invention consists in producing a flow of electric current, preferably by induction, in a definite path in a bath of molten metal and in meanwhile blowing the bath with a gaseous mixture in such manner as to cause a continuous circulation of the metal in a path corresponding to the path of flow of the electric current, the composition of the gaseous agent being such as to assist in the desired refining operations of the bath.

Another feature of the process consists in 35 partially refining the metal or alloy in the usual manner in a converter and then electrically heating the bath in said converter, meanwhile blowing the bath with a gas or gaseous mixture, preferably consisting 40 wholly or in part of the exhaust gas from the converter.

The apparatus of my invention consists of a furnace, such as a converter, provided with means for producing electric heat localized 45 at a particular place or in a particular path in the furnace, and also provided with tuyers arranged to direct a current of gas into the bath in such direction as to produce a circulation of the metal from the less heated 50 portions of the bath to the point of application of the electrically produced heat.

In its preferred embodiment, the apparatus 55 comprises a converter, preferably of the Bessemer type, modified to provide, additional to the main chamber, one or more auxiliary heating chambers, the metal in such

latter chambers being preferably heated by electric currents induced therein, and tuyers being provided to blow a gas in such direction as to cause a continuous circulation between the main and auxiliary chambers. Means are provided whereby the tuyers may receive exhaust gas from the converter, which may be mixed with air or other gases when desired, or said tuyers may be wholly disconnected from the source of exhaust gas and connected to any other convenient source of suitable gas or gaseous mixture. The auxiliary chamber or chambers are preferably so arranged that when the vessel is tilted the entrance of slag into said chambers is prevented.

These and other features of my invention may be more readily understood by reference to the accompanying drawings, in which,

Figure 1 is a section, on the line 1—1 of Fig. 2, of a Bessemer converter modified in accordance with my invention; Fig. 2 is a section on the line 2—2 of Fig. 1; Fig. 3 is a front elevation of the apparatus; Fig. 4 is a horizontal sectional view of an open-hearth furnace modified in accordance with my invention; Fig. 5 is a side elevation, partly in section, of the furnace shown in Fig. 4; Fig. 6 is a section on the line 6—6 of Fig. 5; Fig. 7 is a section on the line 7—7 of Fig. 8 of a well known type of induction furnace provided, in accordance with my invention, with tuyers arranged to blow a gas in a direction to produce a circulation of the metal from the main chamber through the induction channels; and Fig. 8 is a section in the line 8—8 of Fig. 7.

Similar letters of reference refer to similar parts throughout the several figures of the drawing.

Referring more particularly to Figs. 1, 2 and 3, the furnace as shown consists essentially of a standard bottom blow converter vessel 1, the tuyers 2 being arranged in the usual manner to blow a gas into the bath 3 inclosed in the main chamber 4. The converter is modified, however, to permit both of electric heating of the metal refined therein and of utilizing gas as a circulating and treating agent. Communicating at its opposite ends with the chamber 4 is a channel 5, which forms the secondary of an induction furnace. The primary winding 6 of the induction furnace is arranged in one of the several well known methods about the trans-

former core 7. The location of this coil forms no part of the present invention. In short the converter 1 has an induction furnace 8 attached thereto, in such manner that 5 the channel 5 of the induction furnace communicates with the chamber of the converter. In the drawings two channels 5 are shown which merge into a common channel 9, such arrangement being suitable for a 10 two-phase system. Obviously the arrangement may be modified to provide for other types of multiphase induction furnaces.

Twyers 10 are so arranged as to blow gas into the metal or bath in such direction as to 15 produce a circulation of the metal between the channels of the induction furnace and the main chamber. Such twyers 10 are preferably located, as shown in Fig. 1, above the mouth of the channel 9 and are inclined 20 downwardly toward the surface of the bath. The impact of the gas blown through the twyers 10 upon the surface of the bath is such as to entrain the metal and produce a circulation of the molten bath in a general 25 direction such as is indicated by the arrows in Figs. 1 and 2.

The vessel 1 is mounted in the usual manner upon hollow trunnions 11. When the vessel is tilted, as shown in Fig. 1, the channels 30 of the induction furnace are completely filled with metal and the entrance of corrosive slags into said channels prevented. The tilting of the vessel also permits of the adjustment of the distance and inclination of 35 the surface of the bath with respect to the twyers 10.

The mouth 12 of the converter communicates with a pipe 13, which is removably connected to the mouth 12 and which carries 40 off the exhaust gases from the converter for subsequent utilization. The pipe 13 is journaled to swing in a bearing 14 which is in axial alignment with the trunnions, in order that said pipe may swing with the converter.

45 The pipe 13 communicates with a pipe 15 which conducts the exhaust gas through one of the regenerators 16, and from thence through the other regenerator to the pipe 17. The pipe 15 is provided with two 50 valves, one extending to each of the regenerators 16, one of said valves being open while the other is closed, thus controlling into which of said regenerators the gas will first flow. Suitable suction apparatus, as 55 for example a blower, is inserted between the two regenerators to assist in the passage of the gas from the one to the other. The exit pipes from the regenerator to the pipe 17 are provided with valves, one of which is 60 open and the other closed, the valve in the exit pipe from the regenerator through which the gas first flows being closed, while the valve in the other exit pipe is open. The function and operation of these regenerators are well understood and hence a de-

tailed description thereof is unnecessary. The exhaust gas from the converter will consist largely of carbon monoxide, and each regenerator is preferably provided with a valve controlled pipe 16<sup>a</sup> for the admission of air to the regenerator if so desired. Exhaust pipes 18 may also be provided to draw off the surplus gas for other use if so desired.

The pipe 17 leads to one of the trunnions 75 11, from which trunnions two branches 19, 20 lead to the twyers 10 and 2, respectively. A valve controlled pipe 21 communicates with the pipe 17 and serves to supply gas from any suitable source to be used in the 80 treatment until the generators 16 furnish a sufficient supply.

As before stated air may be mixed with the gas, such air being admitted by the pipes 17. If desired the air for the top-blow 85 twyers 10 may be admitted directly into said twyers by a pipe 22, and the gas from the pipe 17 be supplied in the injector principle, the relative proportions of the mixture being controlled by the speed of the blower 23. 90

As shown in Fig. 3, the pipes 19 and 20 are controlled by valves 24 and 25, respectively, in order that either or both sets of bottom and top blow twyers may be utilized in the blow, as may be desired. Furthermore, I preferably provide means whereby 95 an air blow only may be employed in the usual manner, if desired, and for convenience of illustration a separate valve-controlled pipe 26 is shown connected to the 100 other trunnion 11. This construction may also serve for admitting a mixture of reducing gas and air simultaneously into the bath from below.

Figs. 4, 5, and 6 illustrate the open-hearth 105 type of furnace modified in accordance with my invention, two sets of induction furnaces 8<sup>a</sup> being shown disposed upon opposite sides of the main chamber 4<sup>a</sup>. In this arrangement also the chambers 5<sup>a</sup> communicate with 110 the chambers 4<sup>a</sup>, and twyers 10<sup>a</sup> are disposed above the mouth of the common channel 9<sup>a</sup>. Any well known system of regenerators 16<sup>a</sup> may be employed. The supply of gas from the regenerators may be drawn on the injector principle from said regenerators by the injector nozzle 28 supplying air or other 115 suitable gas under pressure. Gas from any convenient source and having any suitable composition may be supplied to the twyers 120 9<sup>a</sup> by the pipe 29.

Figs. 7 and 8 illustrate a well-known type of induction furnace modified in accordance with my invention. In such type of furnace it has been found that the metal in the main 125 chamber 4<sup>b</sup> is not sufficiently heated by the heat developed in the channels, and that it is necessary to resort to other expedients for maintaining all portions of the bath at the requisite uniform elevated temperature. By 130

my invention, however, a continuous circulation of the metal from the main chamber into the auxiliary heating channels is effected by the gas blown through the twyers 30. 5 The exhaust gas from the furnace is led out through the pipe 31, and may be utilized in the manner hereinafter described. The gas supplied by the pipe 32 to the wind-box 33 may be there mixed with air or other gas, 10 supplied by the nozzle 34, the relative proportions of the gaseous mixture being controlled on the injector principle, as hereinbefore described.

While I have thus described several types 15 of converters modified in accordance with my invention, I do not wish to be understood as limiting the invention to the specific structure shown, since it is capable of being embodied in other types of furnaces, and, 20 obviously, different arrangements and changes, within the scope of my invention, may be made even with the types shown and described.

While I furthermore do not wish to be understood as limiting the use of the apparatus hereinafter claimed to the practice of any particular process or processes and desire to cover all uses to which the apparatus of my invention may be put, I will now describe certain processes for the practice of which the apparatus is particularly adapted.

The material to be refined is first treated in any known manner in the converter with or without the aid of electric heat and with 35 any suitable gaseous agent for the removal of undesirable oxidizable impurities. After such treatment the bath, heated electrically, is blown with a reducing gas, as for example, the exhaust gas from the converter, for 40 the purpose of further refining the metals, as for example with the view of deoxidizing the metal of the bath, eliminating such impurities as phosphorus and sulfur, and minimizing the loss of metal which may 45 have become oxidized in the previous treatment. This process is especially applicable to the production of low-carbon steel from high-carbon iron. However in the production 50 of such steel, I preferably remove the slag resulting from the initial treatment, since such slag, in case the metal has been treated according to the Bessemer or other similar processes, contains iron oxids which, as is well known, tend to prevent the 55 removal of sulfur from the metal. After such removal of the slag, a basic flux is added to the bath and the molten mass, while electrically heated, is blown with a reducing gas, as above described. Under such conditions 60 sulfur and phosphorus are readily removed even at comparatively low temperatures, as for example, phosphorus at about 1600° C. and sulfur at much lower temperatures.

65 The apparatus is also particularly adapt-

ed to a modification of the hereinbefore described process which consists in first treating the metal which is to be refined, as for example, high-carbon iron, in the usual manner with air or other oxidizing gas in the converter, however, discontinuing the treatment before the completion of the usual blow, thereby quickly removing the larger part of the oxidizable impurities with comparatively little loss of the metal itself by oxidation. The partially treated metal is then electrically maintained at a temperature at which the affinity of oxygen for the contained impurity, as for example, the affinity of oxygen for carbon, is greater than the affinity of oxygen for the metal of the bath. While the metal is thus maintained at the required temperature, it is subjected to the action of a gaseous mixture, composed partly of an oxidizing agent and partly of a reducing agent, suitable for selectively oxidizing the impurity but unsuitable for a like action on the metal or metals of the bath. This latter part of the treatment is that described and claimed in my copending application Serial No. 488,360, filed April 7th, 1909. The reducing gas employed is preferably the exhaust gas from the converter, which gas consists largely of carbon monoxid (CO).

The apparatus of my invention is also well adapted to the treatment of metals and alloys solely by the process described in my hereinbefore mentioned application for Letters Patent. With such apparatus, gas of 100 a suitable composition can readily be obtained by mixing the exhaust gas from the converter with air or other oxidizing gas. Such mixture, in case air is employed, should be in such proportions that the carbon monoxid is in excess of the oxygen. When the gaseous mixture is blown on the surface of the metal the heat of oxidation of CO into CO<sub>2</sub> is radiated into the bath, and the tendency of the endothermic agent CO<sub>2</sub> to lower the temperature of the bath is thereby offset. When the gaseous mixture is used as bottom-blow, the oxidizing gas may then act directly on the element it is desired to oxidize, without the intermediate reaction between the oxygen and the carbon monoxid of the mixture to first form carbon dioxid as in the case of the top-blow. For this reason the bottom-blow is sometimes preferable, since the heat of oxidation 110 is directly transmitted to the bath and such oxidation tends to aid the electric current in heating the bath.

The terms "high-carbon" and "low-carbon" as used herein are relative terms and 125 are not intended to specify any particular percentage of carbon.

What I claim is:—

1. In a metal refining furnace, the combination with a vessel adapted to contain a 130

- 4
- bath of molten metal, said vessel being provided with a main chamber and an auxiliary heating chamber communicating with the main chamber, of twyers arranged to blow gas into said bath of metal in a direction to produce a continuous circulation of the metal from said main chamber through said auxiliary chamber.
2. In an electric furnace, the combination with a vessel adapted to contain a bath of molten metal, of means for producing a flow of electric current in the metal contained in a particular portion of said vessel, and twyers arranged to blow gas into said bath of metal in a direction to produce a continuous circulation of the metal in the path of said flow of electric current.
3. In an electric furnace, the combination with a vessel adapted to contain a bath of molten metal, said vessel comprising a main chamber and an auxiliary chamber communicating with said main chamber, means for producing induced electric current flow in the metal contained in said auxiliary chamber, and twyers arranged to blow gas into said bath of metal in a direction to produce a continuous circulation of the metal from said main chamber through said auxiliary chamber.
4. In an electric furnace, the combination with a vessel adapted to contain a bath of molten metal, said vessel comprising a main chamber and a channel-shaped auxiliary chamber communicating at its opposite ends with said main chamber, means for producing an induced electric current flow in the metal contained in said auxiliary chamber, and inclined twyers arranged above one of the mouths of the channel for blowing gas downwardly upon the surface of the metal.
5. In an electric furnace, the combination with a main chamber adapted to contain a bath of molten metal, of two channels leading from different portions of said chamber and returning thereto through a common channel, means for producing induced electric currents in the metal contained in said channels, and twyers arranged in proximity to the mouth of said common channel.
6. In an electric furnace, the combination with a vessel adapted to contain a bath of molten metal, means for electrically heating the bath at a particular location in said vessel, and twyers arranged to blow gas into said metal at a point at which the electric heat is communicated to the molten bath.
7. In an electric furnace, the combination with a vessel adapted to contain a bath of molten metal, of means for producing a flow of electric current in the metal contained in a particular portion of said vessel, twyers arranged to blow gas into said bath of metal in a direction to produce a continuous circulation of the metal into the path of said flow of electric current, and means for con-
- ducting the exhaust gas from said vessel to said twyers.
8. In an electric furnace, the combination with a vessel adapted to contain a bath of molten metal, of means for producing a flow of electric current in the metal contained in a particular portion of said vessel, twyers arranged to blow gas into said bath of metal in a direction to produce a continuous circulation of the metal into the path of said flow of electric current, means for conducting the exhaust gas from said vessel, admixing it with other gas and conducting such gaseous mixture to said twyers.
9. In an electric furnace, the combination with a main chamber, of a plurality of channel-shaped chambers communicating at their opposite ends with said main chamber, means for producing induced electric currents in the metal in said channels, and twyers arranged to blow gas into said bath of metal in a direction to produce a continuous circulation of the metal from the channels into said main chamber.
10. The combination with a converter of the Bessemer type, of an electric induction furnace communicating with the interior of said converter, and twyers arranged to blow gas into the metal in said converter and thereby to produce a circulation of metal from said converter through the chamber of said induction furnace.
11. The combination with a converter of the Bessemer type, of a multiphase electric induction furnace provided with a plurality of adjoining annular chambers communicating with the interior of said converter the adjacent portions of said annular chambers being in the form of an enlarged common chamber, and twyers arranged above the mouth of said common chamber for blowing gas downwardly upon the surface of the metal in said converter.
12. In an electric furnace, the combination with a bottom-blow converter adapted to contain a bath of molten metal, of an induction furnace having a channel-shaped chamber communicating at its opposite ends with the interior of said converter, and twyers arranged to blow gas into said bath of metal in a direction to produce a continuous circulation of the metal from the channel into the chamber of said converter.
13. In an electric furnace, the combination with a vessel adapted to contain a bath of molten metal, of means for electrically heating said metal, a twyer leading into said vessel, means for conducting exhaust gas from said vessel to said twyer, an injector nozzle opening into said twyer, and means for forcing gas under pressure through said injector nozzle.
14. The process of extracting and refining metals and alloys, which consists in inclosing a bath of molten metal in a suitable

vessel, producing a flow of electric current in a definite path in said vessel, and blowing said bath with a gas in a direction to produce a continuous circulation of the metal in said vessel in a path corresponding to the path of flow of the electric current.

15. The process of extracting and refining metals and alloys, which consists in inclosing a bath of molten metal in a suitable vessel, producing a flow of electric current in a definite path in said vessel, and blowing said bath with a gas suitable for refining said molten metal, said gas being blown into the bath in a direction to produce a continuous circulation of the metal in said vessel in a path corresponding to the path of flow of the electric current.

16. The process of extracting and refining metals and alloys, which consists in inclosing a molten bath of metal and slag-producing material in a vessel provided with a main chamber and an auxiliary heating chamber communicating therewith, electrically heating the metal contained in said auxiliary chamber, blowing said bath with a gaseous treating agent, such blow being so applied to the bath as to produce a continuous circulation of the metal between said main and auxiliary chambers, and meanwhile tilting said vessel so as to prevent the entrance of the slag into said auxiliary chamber.

17. The process of extracting and refining metals and alloys, which consists in inclosing a molten bath of metal and slag-producing material in a vessel provided with a main chamber and an auxiliary heating chamber communicating therewith, electrically heating the metal contained in said auxiliary chamber, blowing said bath with a gaseous treating agent suitable for inde-

pendently heating the bath, such blow being so applied to the bath as to produce a continuous circulation of the metal between said main and auxiliary chambers, and meanwhile tilting said vessel so as to prevent the entrance of slag into said auxiliary chamber.

18. The process of extracting and refining metals and alloys, which consists in inclosing a molten bath of metal and slag-producing material in a vessel provided with a main chamber and an auxiliary heating chamber communicating therewith, electrically heating the metal contained in said auxiliary chamber, directing a current of heat-supplying gas on the surface of the bath in said main chamber in a direction to produce a continuous circulation of the metal between said main and auxiliary chambers.

19. The process of extracting and refining metals and alloys, which consists in inclosing a molten bath of metal and slag-producing material in a vessel provided with a main chamber and an auxiliary heating chamber communicating therewith, electrically heating the metal contained in said auxiliary chamber, conducting the exhaust gas from said vessel, mixing with an oxidizing gas, and blowing the gaseous mixture into the bath in a direction to produce a continuous circulation of the metal between said main and auxiliary chambers.

In witness whereof, I, hereunto subscribe my name this 23rd, day of October, A. D. 1909.

ALBERT E. GREENE.

Witnesses:

GEORGE E. FOLK,  
GEO. C. DAVISON.